



US005171359A

# United States Patent [19]

Megy

[11] Patent Number: 5,171,359  
[45] Date of Patent: Dec. 15, 1992

[54] REFRACTORY METAL SWARF COMPOSITION

[76] Inventor: Joseph A. Megy, C. M. Tech, P.O. Box 495, Corvallis, Oreg. 97330

[21] Appl. No.: 762,507

[22] Filed: Sep. 19, 1991

[51] Int. Cl.<sup>5</sup> C22C 29/00

[52] U.S. Cl. 75/230; 419/10

[58] Field of Search 75/230; 419/10

[56] References Cited

U.S. PATENT DOCUMENTS

3,753,690 8/1973 Emley et al. 75/412  
4,940,572 7/1990 Laundon et al. 423/633

Primary Examiner—Stephen J. Lechert, Jr.

Attorney, Agent, or Firm—Harness, Dickey & Pierce

## ABSTRACT

A clean refractory metal SWARF particle product is made from refractory metal SWARF. The SWARF particles are produced with coolant at a temperature of less than 650° C. to prevent formation of refractory metal oxides and nitrides. The SWARF particles are comminuted to reduce the particle size of the SWARF slivers and to liberate residual coolant. The comminuted SWARF slivers are washed with a displacement wash to remove the bulk of the coolant and subject to a counter-current wash to remove substantially all of the coolant components to produce clean SWARF particles. The clean SWARF particles can be pressed into briquettes and sintered at elevated pressures or mixed with an alkali metal refractory metal halide salt, pressed at elevated pressures into SWARF/salt briquettes and dried. The briquettes are non-pyrophoric.

8 Claims, 4 Drawing Sheets





FIG. 1



FIG. 2



FIG. 3



FIG. 4

## REFRACTORY METAL SWARF COMPOSITION

## BACKGROUND OF THE INVENTION

This patent relates to a process to convert slivers and fines (referred to as "SWARF" in the industry) from refractory metal (titanium and zirconium metal) belt grinding operations into a consolidated, safe to handle, raw material suitable for aluminum, magnesium and iron refractory metal master alloys, such as aluminum-titanium alloys, magnesium-zirconium alloys, aluminum-zirconium alloys, iron-titanium alloys, iron-zirconium alloys, aluminum-titanium-boron alloys, and the like. At present, most refractory metal products are produced from large ingots, which involve various hot forging and rolling operations. Whenever refractory metals are heated above about 700° C. in air, refractory metal oxides and nitrides are formed with large heat release varying in thickness depending on both the temperature and time. Most of the oxide is removed by 15 mechanical means, usually sand or bead blasting. However, some of the oxide is in the form of pits which projects more deeply than average into the base metal and is not removed by these operations. The pits are usually removed by belt grinding processes in which a silicon carbide, zirconium oxide, or other hard grit, typically about 60 mesh, bonded to a belt is moved over the surface of the metal, removing a mil to several mils of the surface per pass in the form of small curved slivers of the refractory metal. The belt grinding machine 20 gouges the slivers of metal with each of the individual grains of grit on the belt. These fine slivers of refractory metal in bulk are called "SWARF" in the industry. The amount of SWARF generated is perhaps on the order of 25 one percent of the weight of the metal piece being processed, depending on the thickness of refractory metal being ground.

At the present time, SWARF is considered a waste product and is disposed of by burning in the open air at a remote site. SWARF has a very low ignition point and 30 is highly pyrophoric; it combusts suddenly and violently with the rapidity and brightness of a photographic flashbulb to produce a very hazardous fire. Accordingly, SWARF must be maintained under water or under a non-oxidizing environment to reduce reaction with N<sub>2</sub> and O<sub>2</sub> in the air. This burn operation generates a thick white smoke (TiO<sub>2</sub>) or (ZrO<sub>2</sub>) and is receiving increasing scrutiny from regulatory agencies.

The existing grinding operations are conducted with water or a non-flammable grinding fluid (collectively "grinding fluid"). The SWARF is removed from the grinder mechanically along with the grinding fluid. The SWARF and grinding fluid go through an initial screening wherein the coarse SWARF is separated from the bulk of the fines SWARF and the grinding fluid. The SWARF fines and grinding fluid are sent to a filter 45 wherein the SWARF fines are separated from the grinding fluid. The grinding fluid is recycled back to the grinding operation. The coarse SWARF and fine SWARF are combined and disposed of by burning.

The grinding fluid usually contains components to aid in continuously cleaning the SWARF from grinding media and fire retardants. These components also unfortunately add chemical impurities to the SWARF material tending to further limit its value.

The refractory metals titanium and zirconium are made from relatively cheap and plentiful ores. The extraction, purification and consolidation of these met-

als is, however, expensive. Thus the metallic value in the SWARF after its removal during grinding is sufficient to warrant recovery if it can be reprocessed to eliminate its hazardous, pyrophoric nature and cleaned 5 of components detrimental to potential end uses.

## SUMMARY OF THE INVENTION

The present invention is directed to a process for producing a refractory metal product prepared from refractory metals SWARF by treatment of the SWARF from the initial stages of its production.

In one embodiment of the present invention, clean comminuted refractory metals SWARF particles are prepared from refractory metal grinding operations, typically strip refractory metal grinding operations, comprising the steps of:

conducting the refractory metal grinding operation with sufficient grinding fluid or coolant to prevent the produced SWARF refractory metal slivers from exceeding a temperature of some 650° C.;

commuting the SWARF with adherent coolant from the grinding operation to reduce the SWARF refractory metal elongated slivers to refractory metal SWARF particles having length to width aspect ratios substantially less than the elongated slivers, the reduction is accompanied by a reduction in bulk volume of the SWARF and the release of adherent coolant;

separating the refractory metal SWARF particles from the released coolant; and

washing the refractory metal SWARF particles with clean water to yield clean refractory metal SWARF particles.

Preferably before the SWARF with its adherent coolant is comminuted, the SWARF from the grinding operation is separated from the excess coolant. Preferably the SWARF and coolant are first screened to remove the coarse SWARF with some residual coolant from the fine SWARF and the excess coolant. The excess coolant is filtered from the fine SWARF to separate the fine SWARF with some adhered coolant from the bulk of the coolant which is recycled back into the grinding operation.

During the comminuting stage, the bulk volume of the SWARF is dramatically reduced to less than 50% of its pre-communited volume. The comminuting also releases a substantial amount of the adherent coolant, that is, coolant adhering to the SWARF refractory metal elongated slivers. The released adherent coolant separated from the SWARF particles is preferably recycled back to the grinding operation. Preferably, the washing of the SWARF particles comprises at least a displacement wash with water followed by filtration. The displacement wash removes a substantial amount of the remaining adherent coolant which can be recycled back to the grinding operation. In a preferred embodiment, the filtered SWARF particles following the displacement wash are subject to at least three counter-current washes with water. The SWARF particles become cleaner with each succeeding wash and the washing fluid becomes progressively more contaminated with each wash. The washing fluids from the counter-current wash can be used as a displacement wash fluid.

The clean SWARF particles after the final wash can 65 be disposed of as SWARF is presently disposed of, that is, by burning. Preferably, however, the clean concentrated refractory metal SWARF particles are pressed in conventional pressing equipment into SWARF bri-

quettes or other formed body shapes (collectively "briquettes") which reduces the SWARF void volume by at least a factor or two. The SWARF briquettes are then sintered by heating the briquettes to temperature between 800° C. and 1100° C. under a vacuum or under an inert gas atmosphere, such as a helium gas atmosphere or argon gas atmosphere, for a period of time, such as one-half hour, sufficient to sinter the refractory metal in the briquettes to form sintered SWARF briquettes. Preferably the sintering is done at about 950° C. The briquettes have far less void volume and far less surface area than the clean concentrated refractory metal particles. The sintered briquettes are not pyrophoric, they will not burn in the presence of air. In contrast, compacted SWARF sliver briquettes are pyrophoric and such briquettes must be stored under water or stored in an inert atmosphere or vacuum to prevent dangerous combustion.

In the preferred embodiment of the present invention, the clean concentrated refractory metal SWARF particles are processed into a pyrophoric safe refractory metal/salt briquettes. The clean concentrated refractory metal SWARF particles, in a moist state, are mulled with an alkali metal halide salt type to produce a refractory metal/salt mixture. Sufficient alkali metal halide salt type is employed in the mixture to render the refractory metal/salt briquette product pyrophoric safe.

The refractory metal/salt mixture is pressed into refractory metal/salt briquettes; and the refractory metal/salt mixture briquettes are dried to produce dried refractory metal/salt mixture briquettes.

The clean refractory metal SWARF particles are mixed with about 30% to about 100% by weight of the metal with the alkali metal halide salt types. Thus, the dried refractory metal/salt mixture briquettes will comprise from about 23% to about 50% by weight salt with the balance being the refractory metal.

The alkali metal halide salt type can be an alkali metal refractory metal halide, such as sodium titanium fluoride, potassium titanium fluoride, sodium zirconium fluoride, potassium zirconium fluoride or the like. The salt type can also be an alkali metal halide, such as sodium fluoride, potassium fluoride, sodium chloride, potassium chloride and the like. In addition, the alkali metal halide salt type can be a sodium boron fluoride, potassium boron fluoride and the like. Preferably the alkali metal halide salt type is an alkali metal refractory metal fluoride salt wherein the refractory metal is the same as the refractory metal in the master alloy. For example, if the master alloy is to be an aluminum-titanium alloy, the preferred salt type would be an alkali metal titanium fluoride salt. If the master alloy contains boron in addition, preferably the alkali metal halide salt type will be a mixture of salts wherein one of the salts will be an alkali metal boron fluoride salt. The weight ratio of boron to the refractory metal in the salt mixtures should be the same weight ratio of the boron to refractory metal in the master alloy.

Both the refractory metal Ti and Zr particles and the Ti and Zr salts in the refractory metal/salt briquettes will report to the aluminum master alloy. The salt appears to serve as a flux which aids in the dissolution of the refractory metal particles into the aluminum, magnesium and iron master alloy. When the master alloy contains boron, the refractory metal in the Ti salts reacts with the boron salt to form TiB<sub>2</sub> alloy which reports to the aluminum master alloy. The TiB<sub>2</sub> alloy has grain refining properties in aluminum metal. The boron

salt must react with a refractory metal salt to produce a TiB<sub>2</sub> alloy. The bulk refractory metal has mass transfer problems in forming the TiB<sub>2</sub> phase; thus the TiB<sub>2</sub> phase is formed with titanium and boron salts.

Thus, the pyrophoric safe refractory metal/salt briquettes can be utilized to furnish the master alloy with refractory metal or refractory metal and boron, if boron is present in the master alloy. It appears that the SWARF refractory metal in the briquette functions as a scavenger for the iron master alloy by consuming oxygen and nitrogen present in the alloy.

The refractory metal/salt mixture briquettes are dried so that the briquettes can be safely added to the master alloy. If appreciable moisture is retained in the briquettes, the moisture in the briquettes upon contact with the hot, molten master alloy reacts with the molten metal to form hydrogen which is hazardous.

#### BRIEF DESCRIPTION OF THE DRAWINGS

FIG. 1 is a block diagram showing a conventional method of producing SWARF improved according to the present invention;

FIG. 2 is a block diagram showing the improved method of the present invention of producing clean SWARF particles;

FIG. 3 is a flow sheet of the process of the present invention for treating SWARF; and

FIG. 4 is a flow sheet of the counter-current washing step for the process of FIGS. 2 and 3.

#### DETAILED DESCRIPTION OF THE PREFERRED EMBODIMENT

The process of the present invention is applicable to many different alloys of titanium and zirconium. Refractory metals herein means titanium and zirconium metal and/or alloys.

Referring to FIG. 1, a grinding belt having a flexible fabric backing coated with silicon carbide or zirconium-titanium oxide grit, typically about 60 mesh, is used to 40 grind the surface of a refractory metal strip. SWARF can also be produced when surfaces of refractory metal slabs or plates are surface ground. The belt (not shown) is typically two to four feet wide and is looped over two rolls (not shown) approximately three inches in diameter, one of which is powered to rotate the belt at high speed. In operation the sheet, billet, or strip of refractory metal is passed under the moving belt with an operator controlling the pressure between the grinding media and the metal. The point of contact between the grinding media and the refractory metal surface is sprayed with grinding fluid. The fluid is mostly water. Other components include a water soluble oil, and other components such as nitrates, phosphates, organic amines, etc. which aid in keeping the grinding media clean, reducing the pyrophoric nature of the SWARF, and reducing the surface tension of the water.

The first step in the process of recovering SWARF, according to the instant invention, is to prevent excessive reaction of the SWARF with air in the grinding operation itself, which would cause the formation of refractory metal oxides and nitrides. Formation of the refractory metal oxides and nitrides is due to reaction with air at elevated temperatures experienced during the grinding operation. The temperature at which reaction with oxygen and nitrogen is rapid is 650° C. One step of accomplishing this goal is by using sufficient quantities of grinding fluid during the grinding operation to act as a coolant to prevent SWARF from reach-

ing a temperature of 650° C. or more. Preferably sufficient grinding fluid (hereinafter "coolant") is used to prevent the coolant from reaching its boiling point temperature in the grinding operation. During the grinding operation, the grinding belt comes in contact with a large area of the refractory metal sheet or plate. The temperature of the SWARF in this contact area varies depending upon a number of factors. The localized temperature of the SWARF must be maintained below 650° C. This is best accomplished by flooding the grinding area with grinding fluid to maintain the SWARF temperature below 650 C. Sufficient quantities of coolant are used to keep the SWARF particles awash in coolant and to prevent the coolant temperature from reaching its boiling point temperature within the grinding contact area. When the coolant temperature in the grinding operation is kept below its boiling point temperature, little, if any of the refractory metal SWARF reaches a temperature of 650° C. and the refractory metal SWARF does not react with the coolant water to produce hydrogen and refractory metal oxides.

Water based coolants are preferred due to their high heat capacity. However, other types of coolants can be used. Since the use of aqueous grinding fluid during the grinding operation is current practice, the improvement herein lies in using sufficient fluid as a coolant to prevent the SWARF from reaching 650° C. and reacting with oxygen and nitrogen to form oxide and nitride refractory metal impurities.

In a typical grinding operation, a refractory metal strip is introduced to the grinder from a coiler/uncoller combination. These coils are typically 200 to over 1000 feet in length and vary in width from about two to four feet. The strip is ground on both sides in multiple passes until, by visual inspection, the grinder operator determines that surface flaws have been reduced to an acceptable level. The coils are weighed before and after grinding. Records of the weight changes are maintained.

During the grinding operation, the SWARF is continuously removed from the grinder mechanically, falling into troughs along with the coolant. The solid-liquid mixture is moved down troughs by circulating rakes and the excess coolant and SWARF are separated by filtrations. The coolant is recycled to the grinding operation.

In a conventional SWARF grinding process (such as shown in FIG. 1 without the temperature control during grinding), the SWARF and excess grinding fluid are screened to separate the coarse SWARF and residual grinding fluid from the SWARF fines and excess grinding fluid. The SWARF fines and residual fluid are separated from the excess fluid by filtration. The excess grinding fluid is recycled back to the grinding operation through a clean tank to permit settlement of entrained solids. The grinding fluid is moved from the tank to the grinding operation as needed. Grinding fluid make-up is added as necessary. These steps are shown in FIG. 1.

Freshly produced SWARF retains appreciable amounts of coolant and thus has a high moisture content, normally in excess of 50%. Indeed, some moisture levels have been measured at 66%. The present practice in the industry at this point is to collect the SWARF in separate bins. The collected SWARF is periodically removed, transported to a remote site, allowed to dry somewhat, and burned in spectacular fires in the open. The burn is extremely rapid and violent, and it gener-

ates copious clouds of titanium or zirconium oxide dust and combustion products of the agents in the coolant.

Referring to FIG. 2, zirconium slab is fed to a slab grinder wherein the surfaces of the slab are ground, normally one at a time, with abrasive belts in the same fashion as the titanium strip was ground in the strip grinder of FIG. 1. The grinding operation is flooded with sufficient coolant to keep the SWARF awash and to prevent the coolant from reaching its boiling point temperature. This flood cooling substantially prevents the Zirconium SWARF from reaching 650° C. during the grinding operation and reacting with air to form oxide and nitride contaminates.

The SWARF and coolant are passed to a mill wherein the SWARF is comminuted to reduce the size of the SWARF slivers. The comminution reduces the SWARF bulk volume by at least half. The excess coolant is separated from the comminuted SWARF and recycled to the grinding operation via the clean tank.

The comminuted SWARF which has residual coolant is subject to a displacement wash with water or other wash solvent to remove a substantial portion of the remaining residual coolant. Conveniently the displacement wash is conducted on the filter. In a displacement wash, the comminuted SWARF is washed with an equal volume of water or other wash solvent. Surprisingly, the wash fluid after separation from the washed SWARF is slightly diluted coolant which can be recycled to the grinding operation via the clean tank. When the displacement wash is conducted on a filter, the wash fluid is separated from the washed SWARF by filtration. The SWARF and wash fluid can be separated by other conventional means, such as settling and decantation, centrifuge separation, screening and the like.

The comminuted SWARF, after separation from the displacement wash fluid, is preferably counter-current washed as described infra with regard to FIG. 4. The clean SWARF particles can be treated as described below to produce sintered SWARF briquettes or dried SWARF/salt briquettes.

Referring to FIG. 3, in the process of the present invention, the SWARF fines after separation from the excess coolant are combined with the coarse SWARF and subjected to a comminution operation where the elongated slivers of refractory metal are broken up into shorter rods. This operation is conveniently carried out with an intensive mixer with additional mixing paddles.

The average aspect ratio of the SWARF particles as produced in the grinding operation is from 20:1 to 200:1. An intensive mixer can readily reduce the aspect ratio below 5:1. This operation results in a considerable change in the bulk density of the SWARF by increasing the packing volume. Whereas the SWARF as produced has a bulk density similar to steel wool or a Brillo Pad, the comminuted SWARF has a bulk density on the order of about 0.3 g/cc and assumes the characteristics of a metal sludge. This order of magnitude change in bulk density greatly facilitates the safe storage and shipping of the material, and as described below, the recovery of coolant therefrom.

When the SWARF is in the low bulk density state, it can hold up to twice its weight of coolant without having any free liquid. In this state, it acts like a sponge. To cover SWARF in this form, it takes about ten times its weight in water or coolant. When the SWARF is comminuted, a substantial portion of the adherent coolant is released.

Once the SWARF has been converted to the high density form as described above and drained of the freed adherent coolant, the retained coolant is about 40% by weight of the metal. Thus over 70% of the coolant which is otherwise lost with the SWARF under existing practice can be recovered and recycled to the grinding operation. An additional amount of coolant, 15% by weight of the metal, can be recovered by displacement and counter-current washing of the comminuted SWARF. Saving in the cost of coolant is significant and can justify the processing of the SWARF, however, the comminuted SWARF has other advantages. First, it has much higher bulk density reducing the cost of storage and shipping. Second, much less water is necessary to cover the SWARF to eliminate the fire hazard.

After comminuting the SWARF, it is preferably further processed in several wash steps in series, which removes the organic matter and inorganic salts, such as nitrate or phosphate salts, that are common components of the coolant used in the conventional grinding operations. If not washed off, the coolant presents a major source of oxygen, nitrogen, and carbon in the SWARF product. Washing also tends to remove some of the grinding media or grit which has disengaged itself from the belt during the grinding process. The washing is conveniently done with water although aqueous solutions, organic solvents and the like can be used.

The comminuted SWARF is first washed with a displacement wash of water. The comminuted SWARF is separated from the displacement wash water, usually by filtration. This wash step is normally carried out in the filtration apparatus. Surprisingly, the filtrate is similar to undiluted coolant with respect to composition and concentration and can be recycled to the grinding operation.

The counter-current wash is carried out in at least three (3) stages. Referring to FIG. 4, the SWARF particles from the displacement wash is passed to the first wash stage wherein the SWARF particles are washed with the wash solvent from the second wash stage. Preferably the washing in each stage is intensive to remove contamination entrapped in the SWARF matrix and the SWARF slivers. The SWARF particles are separated from the wash solvent and passed to the second stage where the particles are washed with wash solvent from the third stage. The wash solvent from the third stage can be disposed of in an environmentally sound way or, preferably, it can be passed to the displacement wash stage wherein it is used as the displacement wash. After the SWARF particles are washed in the second wash stage, the particles are separated from the wash solvent and passed to the third wash stage where the particles are washed with fresh wash solvent. The wash solvent from the second wash stage is passed to the first wash stage. After the particles are washed in the third wash stage, the clean SWARF particles are separated from the wash solvent and burned as waste material or, preferably, pressed into briquettes and sintered, or mixed with an alkali metal halide salt type, pressed into briquettes and dried. The wash solvent from the third wash stage is passed to the second wash stage.

In counter-current washing, the SWARF particles as they are cleaned from stage to stage are washed with cleaner solvent. This type of washing substantially removes coolant components from the SWARF.

Following the washing process, it is necessary to insure that all of the SWARF remains wet to prevent fire. The wet SWARF is preferably mixed with refractory metal alkali metal fluoride salts in ratios consistent with the ratios of refractory metal in the master alloy. For example, if the master alloy contains 5% by weight titanium and 2% by weight boron, the salt mixture would be formulated to have a 5:2 weight ratio of titanium and boron. For making aluminum-titanium or aluminum-titanium-boron master alloys as an end product, then potassium titanium fluoride, potassium boron fluoride, and titanium SWARF are mixed in ratios appropriate to the end product, as will be explained.

An analogous mixture can be made to produce aluminum-zirconium, magnesium-zirconium, iron-titanium, and iron-zirconium master alloys. For preparation of magnesium-zirconium master alloys, mixtures of potassium zirconium fluoride or sodium zirconium fluoride and zirconium SWARF are useful. For producing products requiring the refractory metal component only, mixture of the SWARF with potassium aluminum fluoride for the aluminum master alloy manufacturing process has been found effective.

Both alkali metal refractory metal fluoride salts and bulk refractory metal, usually in the form of sponge or scrap, is available for use with the SWARF. The instant process permits the heretofore unused SWARF to be used in the alloy industry as a getter for O<sub>2</sub>, N<sub>2</sub> and C and as a grain refiner.

The SWARF is mixed with the alkali metal refractory metal fluoride salts with sufficient mixing to insure that the surfaces of the SWARF, which are quite extensive due to the small average size of the SWARF, are completely wetted with the salt. The wet, alkali metal refractory metal fluoride salt-laden SWARF is then preferably compressed to a convenient size. High compressive forces should be used, such as 5000 pounds per square inch (psi) or more. The wet SWARF alkali refractory metal fluoride mixture may be compacted with conventional equipment. Useful devices include die and mold presses, briquettes, and corrugated and smooth roll presses, and the like. This step squeezes out much of the wash water from the SWARF/salt mixture. Once compressed, the briquette has some structural integrity due to the deformation and interlocking of the SWARF particles with each other.

The compressed SWARF/salt mixture forms a SWARF/salt compacted mass unit which is preferably dried. The compacted mixture can be dried in conventional equipment, such as tray driers, belt driers, etc. Although a direct flame is preferably avoided, an indirect flame can be used to dry as the compacted SWARF/salt mixture is not flammable if it has 23% by weight salt on a dry basis and will not sustain combustion even if heated to red heat under a torch. For SWARF/salt compacted mass units having less than 23% by weight salt on a dry basis, burning may occur, but at a slow, controllable rate. The drying in conventional equipment is heat transfer limited and no "bound water" or "difficult to remove water" is observed. As the SWARF dries, water leaving the mass unit leaves a salt residue. Since surface tension acts to cause collection of the liquids at points of closest contact between the individual pieces of metal SWARF, the evaporation of the water leaves salt "bridges" attached to the closest points of metal. Salt bridging between very close points of contact form sturdy bonds. Therefore, these "salt bridges" strengthen the compressed briquettes.

The SWARF can be mixed with salt over a wide weight range, such as from 1:2 to 9:1 SWARF:salt on a dry basis. The upper limitation for salt appears to be when the salt content interferes with the structural integrity of the SWARF/salt compacted mass unit and renders it friable or easily broken. The lower limit for the salt content appears to be when the salt present is insufficient to prevent rapid ignition or combustion of the SWARF/salt compacted mass unit. Ten percent salt by weight of the mass unit appears to be around the lower limit.

The SWARF/salt compacted mass unit is surprisingly superior in practice to the commonly used sponge or scrap in master alloys. It dissolves more readily and in higher yield into the molten metal and is more reactive with the other components of a master alloy, for example, boron.

The SWARF/salt compacted mass unit having at least 30% by weight salt is also surprisingly flame resistant and therefore safely handled and stored in air. The substantial and surprising degree to which the admixture of alkali metal refractory metal fluorides salt and SWARF suppress flammability appears to be due to several factors.

First, the alkali refractory metal fluorides arrest the flame propagation reactions in combustion processes. The fluoride in the alkali metal fluoride salts and the alkali metal refractory metal fluoride salts suppresses free radical generation which is an important reaction in the combustion process. Some refractory metal fluoride compounds have, in the past, been used as fire retardants in clothing.

Secondly, the alkali metal refractory metal and alkali metal aluminum fluoride salts mentioned above have melting points at around 650° C., or just below the temperature at which titanium and zirconium allow rapid diffusion of oxygen necessary to sustain combustion. The highly endothermic melting process of the alkali metal refractory metal fluoride salts removes heat from the SWARF, as the salts melt at just below the combustion temperature of the SWARF metal.

Thirdly, once melted, the molten alkali metal refractory metal fluoride salt strongly wets the surface of the SWARF metal with a molten salt film that severely limits transport of oxygen and nitrogen to the metal to support combustion.

Fourthly, the molten alkali metal refractory metal fluoride salt forms a molten film which fills void spaces in the SWARF/salt compacted mass unit which would otherwise transport air to the interior of the compact and to those sites inside the briquette which would otherwise have the air metal mixture appropriate for reaction.

Optionally, table salt, NaCl, or any other alkali metal halide salt, such as potassium fluoride, may be added to the wet SWARF/salt mixture prior to pressing to enhance the economics of the resulting mixture since such salts are cheaper than the refractory metal salt. As can be deduced from the mechanisms outlined above, the addition of an alkali metal non-refractory metal halide salt will assist in accomplishing some of the above objectives. Although sodium chloride melts at about 801° C., and potassium chloride melts at about 776° C., slightly above the temperature where the refractory metals allow rapid diffusion of oxygen, the presence of these salts still acts to retard refractory metal combustion particularly as a eutectic of the alkali metal halide

and alkali metal refractory metal halide salt mixture which melts at a lower temperature than either salt.

Where the manufacture of refractory metal-boron master alloys is of importance, the alkali metal refractory metal fluoride salt may be mixed in proportion with an alkali metal fluoro borate salt. In this manner, the boron is more easily added to the master alloy, and it serves to reduce the flammability of the SWARF compacted mass unit, along with the alkali metal refractory metal fluoride salt. For example, potassium fluoroborate has a melting point of about 350° C., and would similarly melt below the temperature at which oxygen diffusion into the SWARF metal takes place. The melting of the potassium fluoroborate would begin to pull any other salts present into its molten solution early on, and thus perform some of the above factors in an accelerated manner. The addition of potassium titanium fluoride, potassium boron fluoride, and/or potassium zirconium fluoride, optionally with potassium fluoride, an intimate mixture is preferred for preparation of aluminum master alloys.

Once the SWARF/salt compacted mass unit is dried, it can be used in the production of master alloys and/or re-alloying refractory metal. This unexpected result occurs despite the fact that raw, refractory metal with clean surfaces does not normally readily dissolve when added to the master alloy molten mass. The salt rises to the top of the master alloy molten mass and is easily drawn off. It appears the salt "fluxes" the dissolution of the refractory metal SWARF with the molten aluminum.

In another embodiment of the present invention, the clean SWARF particles can be sintered. Once the SWARF is washed, it can be compacted and dried without salt addition. It may be heated rapidly and briefly to between about 950° C. and 1100° C. to cause sintering. Sintering causes some of the individual pieces of the SWARF compacted unit mass to become bonded to each other to form a mass having an even higher integrity than the SWARF/salt compacted unit mass. In addition, the surface area of the SWARF is highly reduced during sintering. Sintering at 1000° C. for four hours is sufficient. However, temperatures between 950° C. and 1100° C. can be used to sinter the SWARF compacted mass unit. The sintering is done under vacuum in an inert gas atmosphere, such as under argon or helium. The resulting refractory metal sintered SWARF briquettes can be used in refractory metal metallurgy.

Traditional sources of refractory metal scrap for the aluminum, magnesium and iron alloying markets have been affected by the introduction of electron beam and plasma beam melting. Previously titanium and zirconium turnings, edge trims, and various other forms produced during the conversion of ingot to finished parts for the aerospace and nuclear markets had high enough impurity inclusion levels to restrict their use as recycle materials. These materials were sold to the alloy markets. Processing these materials in a plasma or electron beam furnace eliminates inclusions and allows them to be recycled to high quality consolidated refractory metal which commands a higher price than the traditional scrap markets. Thus the cost of refractory metal feed materials for the alloy market has risen. The refractory metal sintered SWARF briquettes can be used as feed material in such processes.

Although the process steps disclosed herein are generally applicable to refractory metal SWARF process-

ing, the specific examples given below outline the range of application.

In any operation involving the handling or processing of titanium or zirconium SWARF, safety is a paramount concern. SWARF is classified as a hazardous material, by virtue of its flammability. Flammability of dry titanium SWARF is an important consideration in the design of any recovery process. Although the flammability characteristics of SWARF has not been specifically studied, some data has been accumulated on titanium powders by the U.S. Bureau of Mines and is summarized in the following paragraphs.

Like many metal powders, titanium is capable of forming explosive mixtures with air. The ignition temperature of titanium dust clouds formed in laboratory equipment with different samples of powder ranged from 330° C. to 590° C. The minimum explosive concentration determined in tests was 0.045 ounces/cubic foot. Measurements of maximum pressure produced in explosions of powder in a closed bomb at a concentration of 0.5 oz/cu ft. ranged from 46 to 81 lb/sq in. The average rate of pressure rise in the explosion tests was 250 to 3400 lb/sq in/sec and the maximum rate of pressure rise was 550 to 10,000 lb/sq in/sec. The minimum energy of electrical condenser discharge sparks required for ignition of a dust cloud was 10 millijoules and for an undispersed dust layer the minimum value was 8 microjoules. Some samples of titanium powder could be ignited by electric sparks in pure carbon dioxide as well as in air. At elevated temperatures in some cases titanium was found to react in nitrogen as well as in carbon dioxide.<sup>1</sup>

<sup>1</sup> U.S. Bureau of Mines. RI 3722. RI 4835.

Titanium powder in the form of sludge or in a wet condition can be dried safely in a vacuum drier at a temperature not exceeding 110° C. Mixing or blending of dry powder should be done in an inert atmosphere. Tests indicate that the maximum values of oxygen allowed when using different inert gases to prevent explosion of titanium dust are given in TABLE I.

TABLE I

|                |           |
|----------------|-----------|
| Carbon Dioxide | 0% Oxygen |
| Nitrogen       | 6% Oxygen |
| Argon          | 4% Oxygen |
| Helium         | 8% Oxygen |

Heretofore, SWARF had been labeled as too contaminated to be useful in the metal alloy market. The oxidation of the SWARF slivers by air during their removal in the grinding operation and observation of the tendency of SWARF, even when compacted, to float on top of molten aluminum, magnesium, and iron baths and further oxidize, strengthened this belief. Chemical analysis of the SWARF usually showed it to be high in oxygen, nitrogen, and carbon. Surprisingly, the present inventor found that if sufficient coolant was used during the grinding step, that the SWARF slivers themselves remained substantially free from oxygen, carbon, and nitrogen contamination, and that the SWARF could be freed from the majority of contamination by these elements by washing the coolant off the SWARF with water. By using the process disclosed herein, the coolant could be economically recovered for reuse. The cleaned SWARF could be consolidated for use in alloying markets.

## EXAMPLE 1

Eight hundred grams of as-produced titanium SWARF, having the consistency of steel wool from a

sheet grinding operation in which all of the free moisture was drained, was placed in a food processor with a chopping blade turning at 3600 RPM to comminute the material. In two minutes the SWARF was converted from a low bulk density steel wool-like material to a metal particle slurry. The liquid in the slurry had been entrained in the well-drained SWARF even though it appeared to be reasonably dry. Separate drying tests showed pre-commminuted SWARF to contain 66% volatiles indicating even more coolant is present since the coolant was only 94% water and the coolant additives were non-volatiles.

After the comminuted SWARF slurry had settled, 350 grams of coolant was drained off, having been liberated or freed by the comminution. The remaining SWARF slurry (440 grams) was placed in a Buchner filter and given a displacement wash which removed an additional 116 grams of the coolant. The coolant was removed at essentially full strength and was suitable for recycle to the grinding operation. The remaining SWARF was then intensively washed with two liters of distilled water. The analysis of the as produced titanium SWARF which was dried at 110° C. and the comminuted, washed SWARF which was dried at 110° C. is shown in the following Table II.

TABLE II

|            | AS PRODUCED<br>SWARF | CLEANED<br>SWARF |
|------------|----------------------|------------------|
| Percent Ti | 96.4%                | 99.7%            |
| Percent Si | 0.45%                | 0.12%            |
| Percent C  | 0.85%                | 0.16%            |
| Percent O  | 1.9%                 | 0.38%            |
| Percent N  | 0.42%                | 0.026%           |

These data show that the majority of contamination in SWARF produced with plenty of coolant, can be removed by comminuting and washing with water.

## EXAMPLE 2

The wet, washed titanium SWARF obtained from Example 1 was divided into four samples. Separate samples were mixed with 10%, 30% or 50% by weight of wet (about 15% moist) potassium titanium, fluoride and 50% by weight potassium aluminum fluoride. Each sample was compacted into ten pellets each measuring nominally  $\frac{1}{2}$ " diameter  $\times \frac{1}{2}$ " tall. Ten similar pellets were made of comminuted and washed zirconium SWARF and potassium zirconium fluoride. Blank pellets of both comminuted and washed titanium and zirconium SWARF were also prepared. The pellets were prepared using a Carver press. The compaction into pellets resulted in the expulsion of most of the water in the pellets. The pellets without salt had a residual 15% moisture in the pellet when pressed at 20,000 psi in a  $\frac{1}{2}$ " diameter die. The pellets with salt addition retained 4-10% moisture depending on the amount of salt in the mixture. The pellets were dried in an oven at 105° C. All of the pellets reached constant weight in thirty minutes and none of the pellets showed any indication of bound water by the shape of the drying curve.

Several of the pellets of each sample were subjected to flame tests which were conducted by holding the pellets in a neutral  $O_2-C_2H_2$  flame of sufficient intensity to heat a  $1" \times 1" \times \frac{1}{2}"$  thick steel plate to full red heat in 45 seconds. The test was conducted by placing the test pellet on an 8" wide piece of 316C stainless steel flat

bar and pushing it under a fixed torch burning under constant conditions.

Under these conditions, loose, washed and dried titanium and zirconium SWARF ignited immediately in a bright photo flash fashion. Since considerable heat release occurs during the burning process, any significant accumulation of washed and dried SWARF would be extremely dangerous.

Compacts of uncommminated, washed and dried, zirconium and titanium SWARF ignited on the order of 10 one second and burned in a self-sustaining fashion in about 5 seconds. Compacted, uncommminated, washed SWARF is a dangerous material in any significant accumulation and must be stored under water.

Both zirconium and titanium pellets with mixed salt were much less flammable. Potassium titanium fluoride with titanium SWARF, potassium aluminum fluoride with titanium SWARF, potassium zirconium fluoride with zirconium SWARF all significantly improved flammability resistance. Pellets containing about 50% by weight salt took about 10 seconds to reach a temperature where reaction with air began to occur as evidenced by the white color in the pellet flame. In this case, combustion would not sustain itself when the torch flame was removed. The 30% by weight salt 15 pellets were borderline in their ability to sustain reaction with air when the torch flame was removed, and those with 10% by weight salt sustained reaction with the torch removed, but burned in a controllable fashion and far less readily than the pellets with no salt. Compacted SWARF/salt pellets, containing at least 10% by weight alkali metal refractory metal halide salt could be stored without a water cover. Preferably the SWARF 20 pellets would contain at least 30% by weight salt.

Zirconium and titanium SWARF pellets with 30% 35 and 50% by weight salt of the types given above, were immersed in molten aluminum at 700° C. and held under the surface with a graphite tool. The pellets readily reacted and dissolved into the molten metal. Similar tests run on SWARF compacts without salt addition 40 tended not to dissolve and would simply rise to the surface of the melt when the graphite tool was raised. The salt obviously helped "flux" the dissolution of refractory metal into the aluminum.

#### EXAMPLE 3

Several of the titanium and zirconium SWARF pellets prepared in Example 1 without salt were placed in a vacuum furnace and heated to 1000° C. for four hours. The resulting pellets were reduced in volume by about 40% and had a density of 90% of theoretical. These 50 pellets did not sustain combustion in the torch test described above. These pellets did not readily dissolve in aluminum at 700° C. until a layer of potassium titanium fluoride was added to the top of the molten aluminum which led to ready dissolution of the pellets and also 55 reaction of the titanium salt. These pellets have desirable handling characteristics for charging into titanium melting furnaces.

#### EXAMPLE 4

A visual examination of coarse SWARF shows the material to be highly agglomerated in the form of entangled slivers of titanium metal. The unwashed SWARF has a dull, non-lustrous appearance which is improved 60 by washing. The SWARF sliver length appears to be from about 0.02 millimeters to about 2 or 3 millimeters.

The cross sectional dimension appears to be relatively uniform and is estimated to be less than about 0.01 mm in width.

Grains of dark SiC grit are visible under magnification. The grit is dark, lustrous, irregularly shaped but tending to an oblate spheroid. They do not exhibit sharp facets or fracture surfaces. The grit in the SWARF falls roughly into three categories, including (1) Free grit, (2) Grit that is mechanically trapped in the SWARF tangles, and (3) Grit that appears to be bound to the titanium sliver. The SiC grit may be attached to the titanium by a reaction of the titanium with the SiC.

The distinguishing features of fine SWARF and sludge with respect to coarse sludge is simply the particle size and the absence of large SiC particles. Fine SWARF shows no large, discrete particles of SiC grit. Silicon analysis of this material shows appreciable amounts of silicon. Accordingly, the fine SWARF material and sludge apparently contains silicon carbide fines as well as the titanium fines. The fine SWARF and sludge sample particles are at least one order of magnitude and smaller in size than the coarse material.

What is claimed is:

1. A non-pyrotechnic refractory metal formed body suitable for alloying in refractory metal master alloys comprising a compressed formed body of refractory metal particles substantially free of refractory metal oxides and nitrides and substantially free of grinding fluid components utilized in the production of SWARF, and an alkali metal halide salt type, the formed body comprising on a weight basis from about 10% to about 65% of an alkali metal halide salt type with the balance being refractory metal swarf particles.

2. The refractory metal formed body of claim 1 wherein the refractory metal is titanium and the alkali metal halide salt type is a potassium titanium fluoride salt.

3. The refractory metal formed body of claim 1 wherein the refractory metal is zirconium and the alkali metal halide salt type is a potassium zirconium fluoride salt.

4. A pyrotechnic resistant sintered, pressed refractory metal formed body suitable as a starting material for the production of high-quality refractory metal comprising clean refractory metal SWARF particles substantially free of refractory metal oxides and nitrides and substantially free of grinding fluid components used in the production of the refractory metal SWARF, refractory metal SWARF having been pressed at elevated pressure to produce the formed body and the formed body having been sintered at a temperature between of about 950° C. and 1100° C. for a sufficient time to sinter the refractory metal swarf particles.

5. The refractory metal formed body of claim 4 wherein the refractory metal is titanium.

6. The refractory metal formed body of claim 4 wherein the refractory metal is zirconium.

7. The refractory metal formed body of claim 1 60 wherein refractory metal is titanium and the alkali metal halide salt type is a mixture of potassium titanium fluoride salt and potassium chloride salt.

8. The refractory metal formed body of claim 1 wherein the refractory metal is zirconium and the alkali metal halide salt type is a mixture of potassium zirconium fluoride salt and potassium chloride salt.

\* \* \* \* \*